# EUROPEAN PATENT SPECIFICATION

(11) **EP 0 467 857 B1**
(45) Date of publication and mention of the grant of the patent: **06.03.1996**
(21) Application number: 91830235.7
(22) Date of filing: 30.05.1991
(51) Int. Cl.: C22C 33/02

(54) **Powder metallurgy tool steel**
Pulvermetallurgische Werkzeugstähle
Acier à outils obtenu par métallurgie des poudres

(30) Priority: 17.07.1990 IT 4815090
(43) Date of publication of application: 22.01.1992
(73) Proprietor: CENTRO SVILUPPO MATERIALI S.p.A., I-00129 Roma (IT)
(72) Inventor: Guglielmi, Fabio, Aosta (IT); Barcaro, Giovanni, Roma (IT); Sommovigo, Paolo, Roma (IT)
(74) Representative: Gervasi, Gemma, Dr.

(56) References cited:
- EP-A- 0 076 326
- US-A- 3 117 863
- US-A- 4 249 945
- US-A- 4 276 087
- US-A- 4 880 461
- STAHL UND EISEN, vol. 110, no. 1, 15th January 1990, pages 93-103; S. WILMES:"Pulvermetallurgische Werkzeugstähle - Herstellung, Eigenschaften und Anwendung"

## Description

The present invention concerns PM. More precisely it concerns a composition designed specifically for Hot Isostatic Pressing (HIP) capable of furnishing finished products with very good service behaviour.

Metal cutting tools (hobs, cutters, millers, etc.) are subject to very difficult working conditions so they require very good hardness, wear resistance, cutting capacity, thermal shock resistance, toughness, etc,; some of these qualities are actually in contrast with one another and are not easily attained.

The main types of high-speed steels come under two headings:
- tungsten steels, containing from 10 to 20% tungsten, from 5 to 15% cobalt, smaller quantities of chromium and vanadium, and from 0.7 to 1.5% carbon
- molybdenum steels, containing from 3 to 10% molybdenum, up to 8% tungsten, up to 12% cobalt, from 2 to 5% chromium, from 1 to 4% vanadium and from 0.8 to 1.5% carbon.

In tool steels the main functions of the alloy elements are to increase hardenability, form hard wear-resistant carbides, and maintain hardness during tempering or anyway during heating to high temperatures.

Solidification, cooling and more generally treatment conditions help produce the desired characteristics in the steel by exerting an influence on carbide type and size, morphology and extent of segregation, and microstructure.

The introduction of powder metallurgy has led to relatively easy mastery of segregation and microstructural phenomena, but never the less there remain numerous difficult-to-control aspects which have a bearing on finished-product quality.

Furthermore, modern ultra-high-speed machining practices require tools of extremely high quality, and there is a big loss of production every time work is stopped to change a tool.

Hence the search for improvements in tool quality continues unabated. So far progress has been achieved by employing larger quantities of costly alloy elements such as cobalt and tungsten.

The object of the present invention is to provide a better quality PM tool steel which ensures a considerably longer tool life.

Another object is to improve the productivity of the machines on which the ensuing tools are used.

A further object of the invention is to eliminate or at least limit the use of costly, strategic elements, thus lowering the price of the tools made from the steel concerned.

According to the present invention these objects are achieved by a molten steel having the following composition (%wt): C from 1,50 to 1.85%, Mn from 0.20 to 0.55%, Si from 0,35 to 0.70%, W from 1.50 to 3.00%, Mo from 8.00 to 9.50%, V from 5.50 to 6.50%, Cr from 4.00 to 5,00%, the remainder being iron and impurities. Preferred embodiments are disclosed in the dependent claims 2 to 4.

During atomization the powder cooling rate is between 1000 and 10000°C/s. This results in a powder of excellent chemical uniformity, containing very fine carbide precipitates, which are useful during subsequent treatments, as will be explained below.

The powders thus obtained are subjected to Hot Isostatic Pressing to obtain semis such as round bars or more complex shapes which, in turn, can be worked to obtain the desired finished product. The latter is then heated in a salt-bath at a temperature between 1160 and 1200°C for 3 to 10 minutes, hardened in a salt-bath in the usual way at a temperature between 450 and 600°C and then cooled to ambient temperature. Finally the product is tempered three times in succession at temperatures between 530 and 560°C, then 540 and 570°C and again between 530 and 560°C; each of these treatment lasts for between one and two hours. The purpose of these thermal treatments is to solubilize and reprecipitate the carbides in the best possible way as regards composition, quantity and dimensions for the purpose of the invention. Since the carbides are already in very fine form in the atomized powders, they can be solubilized at relatively low temperatures in the 1160 to 1200°C range without there being any excessive grain growth. The carbides thus obtained are of the M2C-MC type; their maximum diameter is less than 3.5 um, typically being between 0.5 and 2.5 um, and they are present with a volume fraction between 13 and 18%.

The characteristics imparted to the tools by that treatment are usually in line with the highest values encountered in the best known tool steels used, even as regards properties that are antithetic or difficult to combine, such as hardness and toughness. It is precisely this general line-up at high values which renders the quality of these tool far superior to any yet known.

Three steels, CSM1, CSM2 and CSM3, have been prepared as per the present invention. Their compositions and those of three comparable steels already on the market, RIF1, RIF2 and RIF3, are compared in Table 1.

RIF1 and RIF2 represent the best tungsten and molybdenum ingot steels respectively, while RIF3 is the most widely used powder steel.

**TABLE 1**

| Steel | Percent composition (by weight) | | | | | | | |
|---|---|---|---|---|---|---|---|---|
| | C | Mn | Si | W | Mo | V | Cr | Co |
| CSM1 | 1.65 | 0.38 | 0.43 | 1.72 | 8.20 | 6.14 | 4.8 | - |
| CSM2 | 1.71 | 0.35 | 0,60 | 2.35 | 9.20 | 5.80 | 4.51 | - |
| CSM3 | 1.83 | 0.45 | 0.52 | 2.76 | 8.69 | 5.56 | 4.22 | - |
| RIF1 | 1.53 | nd | nd | 12.34 | - | 4.89 | 4.34 | 5.01 |
| RIF2 | 1.12 | nd | nd | 1.60 | 9.72 | 1.15 | 3.70 | 7.87 |
| RIF3 | 1.33 | nd | nd | 6.36 | 4.96 | 3.07 | 4.21 | 8.33 |

The characteristics of the precipitates, in terms of carbide type, diameter and volume fraction, are given in Table 2.

**TABLE 2**

| Steel | Volume Fraction (%) | Diameter (um) | Carbide type |
|---|---|---|---|
| CSM1 | 13.6 | 0.9-2.0 | M2C-MC |
| CSM2 | 16.8 | 1.3-2.3 | M2C-MC |
| CSM3 | 17.3 | 0.8-1.7 | M2C-MC |
| RIF1 | 14.3 | 14-16 | M6C-MC |
| RIF2 | 6.0 | 12-17 | M6C-(MC) |
| RIF3 | 13.0 | 4-7 | M6C-(MC,M2C) |

Table 3 reports hardness and wear resistance, Table 4 cutting capacity (Taylor Test), and Table 5 toughness and thermal shock resistance (HF=Heat-cracking Factor).

The above hardnesses are Rockwell (RCH) at ambient temperature and Brinnell (BH) at 550°C. The Marcelin Wear Resistance Test is a technological test well known to esperts.

In the following table the cutting speeds V20, V40 and V60 in the Taylor Test indicate the cutting speeds in metres/minute to which the tool deteriorates in 20, 40 and 60 minutes, respectively.

**TABLE 4**

| Steel | Cutting Capacity | | (Taylor Test) |
|---|---|---|---|
| | V20 | V40 | V60 |
| CSM1 | 48.9 | 47.3 | 45.8 |
| CSM2 | 47.6 | 45.8 | 45.1 |
| CSM3 | 46.4 | 46.8 | 45.6 |
| RIF1 | 49.8 | 47.4 | 46.1 |
| RIF2 | 46.2 | 44.3 | 42.8 |
| RIF3 | 45.9 | 44.3 | 43.3 |

**TABLE 5**

| Dynamic bending rupture strength and thermal shock resistance | | | |
|---|---|---|---|
| | Rupture strength (MPA) | | HF |
| | Longitudinal | Transversal | |
| CSM1 | 390 | 300 | 11.5 |
| CSM2 | 410 | 305 | 12.1 |
| CSM3 | 400 | 295 | 11.2 |
| RIF1 | 132 | 65 | 66.1 |
| RIF2 | 160 | 85 | 26.9 |
| RIF3 | 420 | 305 | 10.1 |

The rupture strengths, in MPA, given in the above Table are for test specimens cut longitudinally and transversally from the original bar.

The heat-cracking factor (HF) indicates the ability of the material to support rapid thermal cycles, as well as the rate at wich thermal fatigue cracks develop and propagate in said material. This factor is measured in the laboratory by means of a test designed by the proprietor of this invention, the method being as follows:

A test disc of the material concerned is made to rotate and heated by induction so that part of its surface on the maximum circumference is heated to about 800°C. At the same time, half of said circumference is cooled by water sprays so that during every revolution of the test specimen its surface is subjected to a thermal cycle between the heating temperature indicated and about 100°C.

Various test specimens of the same material are tested for 500, 1000, 2000 and 4000 revolutions. They are then ground and examined under the microscope to measure the number, length and penetration of the cracks formed during the test.

For each series of cycles a factor C is determined by the formula:$\text{Cn = r x Lm x Pmax}$ where Cn is the factor C after n cycles; r corresponds to the measured crack density, assessed as the number of cracks per millimetre of length of the circumference of the test piece; Lm is the average length of the cracks, being the sum of the lengths of the cracks divided by their number and Pmax is the maximum depth of penetration of the cracks measured along the radius of the test piece.

The Heat-cracking Factor is then determined by the following formula:$\text{HF = (D1+D2+D3+D4):4}$ where D1 is C₅ₒₒ:500; D2, D3 and D4 are (C₁ₒₒₒ-C₅ₒₒ):(1000- 500), (C₂ₒₒₒ-C₁ₒₒₒ):(2000-1000) and (C₄ₒₒₒ-C₂ₒₒₒ):(4000-2000).

As is evident from the preceding Tables, the steel according to the invention is in line - characteristic by characteristic - with the best products on the market, and it is the only one which maintains all its properties consistently high compared therewith. Precisely because of this singular feature of possessing excellent values simultaneously for all relevent characteristics, the steel as per this invention is found to be of an exceptionally high quality in practical applications that is not encountered in any other steel for the same applications.

Envelope-cutting hobs produced according to the present invention and tested over long periods on high-speed gear-making operations have increased line productivity by 400 to 500%. In particular, hobs with CSM1, CSM2 and CSM3 compositions have repeatedly resulted in the production of up to 12000 very hard quenched and tempered steel gears without requiring sharpening, while the average for RIF3 powder steel hobs is 4000 pieces, which is in itself better than the performance of conventional ingot steel hobs. Hence productivity is improved not only through an increase in the number of pieces produced with the same tool, but even more so through avoidance of tool-change stoppages, which are extremely costly in modern high-speed machining operations.

## Claims

1. Powder-metallurgy tool steel characterized by the following composition (%wt): C from 1,50 to 1.85, Mn from 0,20 to 0.55, Si from 0.35 to 0.70, W from 1.50 to 3.00, Mo from 8.00 to 9.50, V from 5.50 to 6.50, and Cr from 3-00 to 5.00, the remainder being iron and minor impurities.

2. Steel as per Claim 1 characterized by the fact that the powder is obtained by atomization in a gas which may be nitrogen or argon, the ensuing particles being spherical in shape, 80% of them being smaller than 500 um.

3. Steel as per Claim 2, characterized by the fact that after submission to the following cycle:
- cooling during powder solidification at a rate between 1000 and 10000°C/s
- hot isostatic pressing to obtain a semifinished piece
- transformation of the semi into the desired product
- heating of the product in a salt-bath at a temperature betwe en 1160 and 1200°C for between 3 and 10 minutes
- hardening in a salt-bath at a temperature between 450 and 600°C followed by cooling to room temperature
- series of three successive temperings at temperatures between 530 and 560°C, between 540 and 570°C, and again between 530 and 560°C, each for between one and two hours
it contains precipited carbides of the M2C-MC type measuring less than 3.5 um and a volume fraction between 13 and 18%.

4. Steel as per Claim 3 characterized by the fact that the maximum dimension of said carbides is between 0.5 and 2.5 um.

## Patentansprüche

1. Pulvermetallurgischer Werkzeugstahl, dadurch gekennzeichnet, daß seine Zusammensetzung ist (% im Gewicht): C (1,50-1,85), Mn (0,20-0,55), Si (0,35-0,70), W (1,50-3,00), Mo (8,00-9,50), V (5,50-6,50) und Cr (3,00-5,00), wobei das Übrige Eisen und kleinere Unreinheiten ist.

2. Werkzeugstahl nach Anspruch 1, dadurch gekennzeichnet, daß das Pulver durch Zerstäubung in einem Gas erhalten wird, das Stickstoff oder Argon sein kann, wobei die herauskommenden Teilchen kugelförmig sind und 80% von denen kleiner als 500 µm sind.

3. Werkzeugstahl nach Anspruch 2, dadurch gekennzeichnet, daß er nach dem folgenden Zyclus:
- Abkühlung während der Pulvererstarrung mit einer Geschwindigkeit von 1000-10000°C/s;
- Warme isostatische Verdichtung um ein halbfertiges Stück zu erhalten;
- Umwandlung des halbfertigen Stückes in das gewünschte Produkt;
- Erhitzung des Produktes in einem Salzbad mit einer Temperatur von 1160-1200°C für 3-10 Minuten;
- Verhärtung in einem Salzbad mit einer Temperatur von 450-600°C und folgende Abkühlung bis zur Raumtemperatur;
- Serie von drei Anlassen nacheinander, mit Temperaturen von 530- 560°C, 540-570°C und dann wieder 530-560°C, jedes von denen für 1-2 Stunden;
niedergeschlagene Karbiden vom M2C-MC Typ enthält, die weniger als 3,5 µm messen und einen Inhaltsbruchteil von 13-18% darstellen.

4. Werkzeugstahl nach Anspruch 3, dadurch gekennzeichnet, daß die maximale Größe der Karbiden 0,5-2,5 µm ist.

## Revendications

1. Acier à outils obtenu par métallurgie des poudres, characterisé par la composition suivante (% en poids): C (1,50- 1,85), Mn (0,20-0,55), Si (0,35-0,70), W (1,50-3,00), Mo (8,00- 9,50), V (5,50-6,50) et Cr (3,00-5,00), le reste étant fer et petites impuretés.

2. Acier selon la revendication 1, characterisé en ce que la poudre est obtenue par atomisation dans un gaz qui peut être azote ou argon, les particules dérivantes étant sphériques, 80% entre elles étant plus petites que 500 µm.

3. Acier selon la revendication 2, characterisé en ce que, après le cycle suivant:
- refroidissement pendant la solidification de la poudre, à la vitesse de 1000-10000°C/s;
- compression isostatique chaude pour obtenir un produit semi-fini;
- transformation du produit semi-fini dans le produit requis;
- échauffement du produit dans un bain de sel à la température de 1160-1200°C pour 3-10 minutes;
- trempe dans un bain de sel à une température de 450-600°C suivie par un refroidissement à température ambiante;
- série de trois revenus, l'un après l'autre, à températures de 530-560°C, 540-570°C et encore de 530-560°C, chacun pour 1-2 heures,
l'acier contient des carbures précipités du genre M2C-MC qui mesurent moins de 3,5 µm et qui représent une fraction en volume de 13-18%.

4. Acier selon la revendication 3, characterisé en ce que la dimension la plus grande des susdits carbures est 0,5-2,5 µm.
